

Dec. 29, 1964

H. BENDER ETAL

3,163,795

ELECTRON TUBE

Original Filed March 14, 1957



INVENTOR.  
HARRY BENDER  
BY HARRY P KLING

*Theodore J. H.*  
ATTORNEY

# United States Patent Office

3,163,795

Patented Dec. 29, 1964

1

3,163,795

## ELECTRON TUBE

Harry Bender, Albertson, and Harry P. Kling, Wantagh, N.Y., assignors, by mesne assignments, to Sylvania Electric Products Inc., Wilmington, Del., a corporation of Delaware  
Original application Mar. 14, 1957, Ser. No. 646,010. Divided and this application Mar. 29, 1960, Ser. No. 23,593

2 Claims. (Cl. 313—270)

Our invention is directed toward electron discharge devices and more particularly relates to cathodes for use therein. This application is a division of application Serial No. 646,010, filed March 14, 1957, now abandoned.

As is well known to the art, the cathode or electron emissive element of a cathode is conventionally composed of nickel or a nickel-rich alloy. In forming the element which is normally either planar or cylindrical in shape, the nickel or a mixture of nickel and certain well known additives, as for example magnesium or tungsten, are first melted, either in air or in vacuo, to form a billet. The billet is subsequently rolled and annealed to form a sheet from which the cathode elements are subsequently fabricated.

The composition of the cathode must be controlled within extremely close tolerances to prevent impairment of electrical and structural properties. Such control is extremely difficult, both because of these tolerances and further because extensive testing of the final product is necessary to determine whether or not the final product meets the necessary specifications. The rejection rate is extremely high, and a costly process results.

In our attempt to decrease the cathode rejection rate and thus to decrease the costs of producing cathodes, we discovered that, when powder metallurgy techniques were used in the manufacture of cathodes, a much higher degree of composition control was obtained and thus the rejection rate was sharply decreased.

Surprisingly, however, we also discovered that the cathodes so produced exhibited certain previously unsuspected but highly desirable properties. In particular, we found that the strength of these cathodes substantially exceeded that of conventional indirectly heated cathodes, a highly significant improvement in a field where ever increasing emphasis has been placed on the development of stronger cathodes for use in electron discharge devices which are subject to severe vibrations and other types of mechanical stress.

We further discovered that when our cathodes were fabricated into electron tubes and tested, the sublimation of certain additives, such as magnesium, was sharply reduced over that conventionally obtainable, thus minimizing leakage and other factors adversely affected by such sublimation.

It is, therefore, an object of our invention to increase the strength of cathodes.

Another object is to reduce the costs of manufacturing cathodes through use of powder metallurgy techniques.

Still another object is to provide a new process for producing cathodes.

Yet another object is to provide new and improved cathodes, the strength of which substantially exceeds that of conventional cathodes.

Still a further object is to reduce sublimation of metals, such as magnesium, during testing and operation of electron tubes.

2

These and other objects of our invention will either be explained or will become apparent hereinafter.

In accordance with the principles of our invention, pure nickel powder of high purity, with or without trace additives, is rolled into a fragile porous sheet. This sheet is then sintered to form a strong, substantially non-porous sheet which is then reduced to desired dimensions in accordance with conventional rolling and annealing schedules and then fabricated, for example, into planar or

10 cylindrical cathodes.

The composition of cathodes so formed can be so accurately controlled that the compositions of successive batches (within the limits of experimental errors of analysis) have been found to be identical. Moreover, the 15 strength of such cathodes is greatly increased over normal, the collapse strength being on the order of 2 to 3 times as large as that of conventional cathodes. Further, the sublimation rate of our cathodes when inserted into tubes and tested, is reduced by a factor of ten or more 20 as compared to that conventionally obtained.

We found that the oxygen content of our cathodes is substantially in excess of the oxygen content of conventional cathodes, the ratio of the oxygen content of our cathode to that of conventional cathodes having otherwise 25 substantially identical composition ranging from a minimum of about 2 to a maximum of 10 or more.

While it is not our intention to be bound by theory, we believe that this increased oxygen content plays a primary role in the increased strength of our cathodes. More 30 particularly, it is our belief that the oxide which is normally formed about the surface of metal powders is not reduced during rolling and sintering, but rather remains as discrete oxide particles within the sintered sheet. Such particles apparently inhibit grain movement and 35 deformation, thus stiffening and strengthening the sheet structure.

Our invention will now be described in more detail with reference to the accompanying figure which shows an electron tube incorporating one of our cathodes.

40 Referring now to the figure, an evacuated tube envelope 10 is secured to a tube base 12. An indirectly heated cathode containing one of our cathodes in the form of a sleeve or cylinder 18 coated with an electron emissive coating 19 and a folded heater 14 is positioned within 45 the envelope. A grid wire 20 and an anode 22 are also supported within the envelope by mica spacers 24 and 26 which, in turn, are supported on wire supports 30 and 32.

This cathode is fabricated by first thoroughly blending 50 nickel powder of high purity either without additions or with powder additives in the form of metal or intermetallic alloys. The blended powders are then passed through a rolling mill to form a fragile porous sheet. The sheet is then sintered in an oxygen free atmosphere, such as argon or dry hydrogen, at a temperature falling 55 within the approximate range 800° C.-1150° C. until the porosity is greatly reduced and a strong relatively non-porous sheet is produced. We have found that normally a five minute sintering period is sufficient when a firing temperature of 1000° C. is used. The sintering period is a function of the firing temperature and decreases as the temperature increases.

Following this, the sheet is rolled and annealed to desired dimensions in conventional manner and is thereafter formed into tubular or planar cathodes.

We have found that any of our compositions can be produced in any number of successive batches which

within the limits of experimental errors of analysis are identical in composition.

*Example I*

A cathode sleeve was prepared having the following composition:

| Material: | Percent Content by Weight |
|-----------|---------------------------|
| Manganese | 0.184                     |
| Carbon    | 0.006                     |
| Iron      | 0.052                     |
| Aluminum  | 0.003                     |
| Cobalt    | 0.094                     |
| Silicon   | 0.020                     |
| Copper    | 0.015                     |
| Titanium  | 0.004                     |
| Magnesium | 0.112                     |

the remainder being nickel with small amounts of nitrogen, hydrogen and oxygen.

All trace ingredients other than magnesium were present in the high purity nickel powder; the magnesium was added in the form of an intermetallic alloy of nickel and magnesium, the chemical formula being  $Ni_2Mg$ .

The above alloy was analyzed for its gas content and was found to contain 0.001% by weight of nitrogen, 0.001% by weight of hydrogen, and 0.020% by weight of oxygen.

A conventional nickel-magnesium cathode was analyzed and found to contain about 0.0042% by weight of oxygen, all other composition ranges being substantially identical with that of our cathode.

Our cathode and the conventional or control cathode were tested for collapse strength; the control cathode was found to have a stiffness of 460 grams, while our cathode had a stiffness of 578 grams.

Tubes of the type commercially designated as 12BA6 were fabricated using both types of cathodes and were tested. After a complete life test, the two types of cathodes were removed from the tubes and again tested for collapse strength; the control cathode was found to have a stiffness of 180 grams while our cathode was found to have a stiffness of 420 grams.

Emission measurements showed that the emission within tubes having our cathodes was at least equal to that obtained within tubes having the control cathodes.

The conductivity as measured between the cathode and the control of tubes employing our cathodes ranged between 1/10 to 1/100 of the conductivity of tubes employing the control cathode. The conductivity is directly related to the degree of sublimation of the metallic elements other than nickel present within the cathode, and hence this test shows that the sublimation in the control tube is at least 10 times as large as the sublimation in tubes employing our cathodes.

Further tests showed that the oxygen content of our

sleeve could be decreased to about 0.010% by weight or could be increased to about 0.100% by weight without deleterious effect. Reductions in oxygen content below 0.010% by weight resulted in decreased stiffness, while increasing the oxygen content above about 0.100% caused the sleeve to become somewhat brittle although the stiffness was not adversely effected.

While the sublimation of our cathodes when incorporated in a tube was always less than conventionally obtainable, we found that best sublimation results were obtained by maintaining the magnesium content within the range 0.05% to 0.12% by weight.

Both types of cathodes, i.e. our cathodes and control cathodes, were fabricated from pure nickel and tested in the manner indicated. It was found that the emission of both cathodes decreased in the same proportion, the stiffness of both types of cathodes having about the same values as previously indicated.

While we have shown and pointed out our invention as applied above, it will be apparent to those skilled in the art that many modifications can be made within the scope and sphere of our invention as defined in the claims which follow:

What is claimed is:

1. A cathode provided with a nickel substrate and an electron emissive layer in intimate contact with said substrate, said substrate having an oxygen content as expressed in percent by weight of said substrate which ranges between a minimum of about 0.01% and a maximum on the order of 0.1%.

2. An electron discharge device having a cathode characterized by a high collapse strength and low sublimation, said cathode being provided with a nickel substrate and an electron emissive layer in intimate contact with said substrate, said substrate having an oxygen content which ranges between a minimum of about 0.01% by weight of said substrate and a maximum on the order of 0.1% by weight of said substrate.

**References Cited by the Examiner**

**UNITED STATES PATENTS**

|           |       |            |       |           |
|-----------|-------|------------|-------|-----------|
| 1,699,639 | 1/29  | Van Gessel | ----- | 313—346 X |
| 2,543,439 | 2/51  | Coomes     | ----- | 313—346 X |
| 2,566,115 | 8/51  | Bounds     | ----- | 313—346 X |
| 2,657,325 | 10/53 | Homer      | ----- | 313—346   |
| 2,746,741 | 5/56  | Naeser     | ----- | 75—208    |
| 2,814,564 | 11/57 | Hayden     | ----- | 75—214    |

**FOREIGN PATENTS**

700,606 12/53 Great Britain.

DAVID J. GALVIN, *Primary Examiner*.

RALPH G. NILSON, ARTHUR GAUSS, *Examiners*.